

## UNITED STATES PATENT OFFICE

2,211,582

PROCESS OF ELECTROLYTICALLY COATING  
NONCONDUCTIVE MATERIALS

Samuel Ruben, New Rochelle, N. Y.

No Drawing. Application May 6, 1938,  
Serial No. 206,372

7 Claims. (Cl. 204—22)

This invention relates to a process for producing electrically conductive metal surfaces on non-conductive or high resistance materials, and to products made thereby.

5 An object of the invention is the conversion of high resistance surface coatings to highly conductive coatings.

Another object is to provide a method for 10 economically and simply producing thin highly conductive metal surfaces upon insulating bases.

A further object is the provision of an improved method of providing a conductive metal surface on a high resistance base.

15 Another object is the provision of a method which facilitates electroplating of metals.

A further object is the provision of an article of manufacture comprising an insulating base and a conductive surface formed from metal particles joined together to form a low resistance 20 conductive path.

Other objects will be apparent from the disclosure.

The invention comprises the use of an insulating or high resistance base such as mica, 25 porcelain, paper, rubber, cellulose, plastics, etc., a coating of finely divided copper alloy particles held on said base by a binder, the particles being substantially all metal but having high resistance 30 surface layers of superficial thickness practically invisible to the naked eye, and a means for converting these high resistance surfaces to a highly conductive state in situ on the base.

Heretofore several methods have been used to 35 provide electrically conductive coatings on insulating or high resistance bases. By one method, atomized metal is sprayed onto the insulator surface by a "Schoop" gun. By another method, vaporized metal is sputtered upon the insulator 40 surface. Such methods are unsuited for coating certain types of objects such as thin nonmetallic sheets, are expensive inasmuch as they require the use of hydrogen, vacuum or inert atmospheres, and the coatings produced are in a great 45 many cases unsatisfactory due to rigidity and lack of uniformity.

Another method, much used, particularly in 50 the preparation of electrotypes, is to graphitize the nonconductive surface and electroplate a metal over the graphite. While for a number of uses this method is satisfactory, the specific resistance of the carbon or graphite is so high as to preclude the initial use of high current densities in the electroplating process. In addition, as 55 the graphite is not bonded to the insulator, peel-

ing sometimes results with consequent dislodging of the plated metal film.

The art also discloses the application of metal 5 coatings to nonconductive bases by applying finely divided metal and a binder to the base, precipitating a metal layer on the coating as by immersion in a silver or copper plating solution and thereafter electroplating a layer of metal on the precipitated metal surface. However, the deposited conductive coating does not form a continuous sheet, is not bonded to the base and may be readily rubbed off.

The present invention overcomes the difficulties inherent in the prior art methods and provides an improved material at lower cost. The coating 15 produced by my present method results in a low resistance surface, the conductivity of which closely approximates that of metal foil.

In an endeavor to produce a conductive sprayed metal surface upon an insulating or high 20 resistant base which would possess the advantages of a bonded unitary assembly and which would be free of the limitations heretofore encountered in the art, I have found the following:

If an insulator base be coated with a layer of 25 bronze powder, such as a copper 70%, zinc 30% mixture and bonded to the base by means of an organic binding material such as a natural or synthetic resin, lacquer, etc., such a layer has a high insulating value of resistance along its 30 length, notwithstanding the bronze particles are apparently completely metal and in contact with each other. I have found that this nonconductive condition is due to a high contact resistance at the particle interfaces. This high contact 35 resistance, which I have found to be characteristic of flocculent copper base materials, is, I believe, due to an invisible oxide layer of superficial thickness. The additive effect of this multiplicity of inter-particle resistance layers produces the high 40 resistance surface. Even though the binder be present in negligible quantities only, or even without any binder at all, the high resistance or nonconductive quality of the bronze coating still remains and rubbing or rolling will not eliminate 45 the inter-particle resistance. In the present invention I have eliminated the high resistance at the particle boundaries and rendered the coating conductive over its length by exposing the coating to the effects of a suitable acid, preferably 50 hydrochloric acid in vapor form. The effect of this treatment as can be observed and measured, is to eliminate the high contact resistance at the particle interfaces and reduce the superficial oxide surfaces to metal, as a result of which the 55

resistance immediately drops to a very low value. For example, a strip of "Cellophane" one inch wide, six inches long, when sprayed with a bronze lacquer mixture will show a resistance in the order of 50 megohms. After exposure to the vapors from hydrochloric acid the resistance drops to 0.06 ohm and maintains this condition unless heated and exposed to oxygen. Hydrofluoric acid vapor may be used in place of hydrochloric acid vapor but its use in production presents difficulties.

As a base upon which additional layers of metal can be plated, this highly conductive layer allows application of higher current densities than could be applied to the commonly used graphitized surfaces and provides a continuous process for producing sheet material having a heavy electro-deposited metal surface bonded to the nonconductive base. Due to the fact that the resistance of the copper base layer is extremely low, somewhat in the order of copper or brass foil, it is possible to directly plate silver, gold, chromium, cadmium, nickel, etc., without the necessity of providing a preliminary copper coat. As the underlying metal layer is bonded to the base, the plating will not chip or peel.

While exposure to the vapor or gas of hydrochloric acid is the most rapid and preferred treatment, I have also found it possible to convert the bronze coating to a conductive condition by immersing the coated bronze article for several seconds in a suitable acid such as hydrochloric, hydrofluoric, phosphoric, lactic or sulphuric acid, all of which bring about a reduction of the superficial oxide surfaces of the metal particles with resultant low resistance layers. This method requires more care than the vapor method and necessitates washing and drying to clean the surface of acid.

40 In practicing the invention, a copper bronze powder is sprayed on the insulator or high resistance member to a thickness of about  $\frac{1}{2}$  mil, using a quick drying binder such as a solution of 2 ounces of cellulose in one gallon of amyacetate. This solution forms a porous skin between the particles and allows them to be treated. After the sprayed film is dried it is exposed for several seconds to the vapors of concentrated hydrochloric acid and thereafter heated to expel 50 any surface-absorbed acid gas or vapor. The hydrochloric acid vapor reacts with the surfaces of the particles, reduces the cuprous and other oxides thereon, and in the process, some of the zinc which may be present in the bronze, is consumed.

The material as thus produced is suitable for many uses. However, in some cases it may be desirable to reinforce the sprayed surface with an electro-deposited metal. This may be readily 60 accomplished at a higher current density than possible in the electroplating of metals upon graphitized or carbonized surfaces, the low resistance of the sprayed surface making the use of high currents practicable. In part, this superiority to the usual graphite surfaces heretofore used is due to the more intimate bonding of the conductive particles to the insulator surface, the waterproof character of the bronze coating and its lower resistance. Any of the commonly 65 used plating metals may be employed, for instance, copper, chromium, tin, cadmium, lead, etcetera.

There are numerous applications in which the invention may be used such as, for example, in 70 the production of electrostatic speaker dia-

phragms, unitary electrode-dielectric members for electrostatic condensers, the coating of insulated wires to afford a coaxial conductor external to the core, coating of end terminals on electrical resistance units such as carbon type 5 variable resistors, coating by bronze spraying or dipping and subsequent electroplating of shingles, electrotypes, odd shaped bodies composed of insulating materials such as ornamental plastic objects, containers and a large number of other articles, providing electrostatic shields for glass radio tubes (as well as for other radio parts) by coating the glass with bronze lacquer and exposing the coating to hydrochloric acid vapor, etcetera.

The present invention allows the substitution of molded plastics for plated cast metal parts, such as door knobs and handles, etc., with the important advantage that the electroplated metal, such as nickel, silver or chromium has much greater durability due to the absence of corrosion which in most cases is brought about by galvanic action between the plated metal and the dissimilar metal base.

In some cases, as in the preparation of resistance units for radio volume controls, the bronze coating is treated only to the point where the desired resistance value is obtained, the inter-particle contact resistance being only partially reduced.

In coating "Cellophane," ethyl cellulose, cellulose acetate, paper or other sheet material, a continuous process is used, the "Cellophane" being coated with copper bronze lacquer as it is unrolled, being passed through an oven to dehydrate the "Cellophane" and bake the coating, then exposed to the hydrochloric acid vapor, again heated, passed into electroplating bath, thereafter being washed, dried and rewound.

In general, the method described has been found exceedingly useful and superior to present available methods in providing a highly conductive layer on an insulating or high resistance surface.

While I have found a solution of 2 ounces of cellulose to one gallon of amyacetate to be a very satisfactory binder, other materials may be used such as urea formaldehyde resin, shellac, glyptal, meta methacrylate, etcetera. The amount 50 of binder used should be limited so as not to form a complete physical insulating layer around the particles, but should be sufficient to firmly hold the metal particles upon the insulator base. In practice I have used a mixture consisting of 2 55 ounces of nitro cellulose to one gallon of amyacetate to which I add 20% by weight of finely divided bronze powder. When this mixture is sprayed the cellulose film formed around the bronze is porous and allows contact between the particles. 60

For some applications, as in the treatment of "Cellophane" or other sheet materials, the bronze is applied to the sheet by a printing process instead of by spraying. In the printing process, the sheet is first coated with an adhesive such as 65 urea resin and while still tacky it is coated with bronze powder which is brushed and rubbed on by rotary brushes. This coating is similar to the sprayed coating and is extremely high resistant until exposed to the hydrochloric acid vapor or 70 other treatment above described.

This application is a continuation in part of my co-pending applications bearing Serial Number 168,114, filed October 9, 1937 and Serial Number 205,209, filed April 30, 1938.

Having described my invention, what I claim as new and desire to secure by Letters Patent, is:

1. The method of providing a conductive metal coating upon a nonconductive object which comprises applying to said object a coating of copper base particles and a binder, said particles having normally a high resistance oxide layer of superficial thickness at the surfaces thereof, subjecting said coating to a reducing acid vapor reacting with said particles and removing the oxide, and thereby converting said high resistance surfaces to a conductive state, thereafter electroplating a layer of metal over said coating.
2. The method described in claim 1 characterized in that the acid vapor is hydrochloric acid vapor.
3. The method of providing a conductive metal coating upon a nonconductive object which comprises applying to said object a coating of copper base particles and a binder, said particles having normally a high resistance oxide layer of superficial thickness at the surfaces thereof, and thereafter subjecting said coating to the action of a reducing acid chemically reacting with said particles and removing the oxide, and thereby converting the high resistance surfaces thereof to a conductive state, thereafter electroplating a layer of metal over said coating.
4. The method as described in claim 1 characterized in that the reducing acid is hydrochloric acid.
5. The method of providing a conductive metal coating upon a nonconductive base which comprises applying to said base a coating of copper-zinc bronze particles and a binder, said bronze particles having normally a high resistance oxide layer of superficial thickness at the surfaces thereof, and thereafter subjecting said coating to the action of a zinc dissolving reducing acid capable of reacting with said bronze particles and removing the oxide and thereby converting the high resistance surfaces thereof to a conductive state, thereafter electroplating a layer of metal over said coating.

layer of superficial thickness at the surfaces thereof, and thereafter subjecting said coating to the action of a zinc dissolving reducing acid capable of reacting with said bronze particles and removing the oxide and thereby converting the high resistance surfaces thereof to a conductive state, thereafter electroplating a layer of metal over said coating.

6. Continuous process for metal coating nonconductive sheet material of the class comprising "Cellophane," paper and the like, which comprises applying to said sheet a coating of copper base particles and a binder, said particles having normally a high resistance oxide layer of superficial thickness at the surfaces thereof, heating said coated sheet, exposing said sheet to the action of a reducing acid vapor chemically reacting with said particles and removing the oxide and thereby converting the high resistance surfaces thereof to a conductive state, thereafter passing said sheet into an electroplating bath and plating a layer of metal upon said coating, thereafter washing and drying said sheet.

7. Process for the metal coating of shingles which comprises applying to a shingle a coating of copper base particles and a binder, said particles having normally a high resistance oxide layer of superficial thickness at the surfaces thereof, and thereafter subjecting said coating to the action of a reducing acid vapor chemically reacting with said particles and removing the oxide and thereby converting the high resistance surfaces thereof to a conductive state, thereafter electroplating a layer of metal over said coating.

SAMUEL RUBEN.